

Sept. 2, 1941.

E. B. GRAHAM

2,255,006

PISTON FOR INTERNAL COMBUSTION ENGINES

Filed Oct. 5, 1937

2 Sheets-Sheet 1



Fig. 1



Fig. 4

E. B. Graham  
inventor

By: Glascock, Downing, Sebold  
Attns.

Sept. 2, 1941.

E. B. GRAHAM

2,255,006

PISTON FOR INTERNAL COMBUSTION ENGINES

Filed Oct. 5, 1937

2 Sheets-Sheet 2



Fig. 5



Fig. 2



Fig. 3

E. B. Graham  
Inventor

By: Glascock Downing & Debold  
Atty.

## UNITED STATES PATENT OFFICE

2,255,006

## PISTON FOR INTERNAL COMBUSTION ENGINES

Eric Bradley Graham, Friern Park, North Finchley, London, England, assignor to Specialloid, Limited, London, England

Application October 5, 1937, Serial No. 167,462  
In Great Britain September 28, 1936

5 Claims. (Cl. 309—14)

This invention relates to light alloy pistons for internal combustion engines.

It has been found in connection with such pistons that certain advantages are secured by furnishing in the structure of the piston a ring of cast iron or steel of an austenitic character particularly in the case of pistons for compression ignition engines.

Certain prior proposals in connection with light alloy pistons have involved modification of the composition of the light metal alloy and the employment of cast iron of a composition such that the co-efficient of thermal expansion of the latter is substantially the same as that of the light metal alloy, or alternatively, without necessarily modifying the composition of the light alloy by the inclusion thereof of a relatively considerable proportion of silicon to employ an iron alloy having a high nickel content which has a co-efficient of thermal expansion less but not more than 10 per cent, less than that of the material of the piston.

Thus, it is suggested in the latter case that the light alloy may have a co-efficient of thermal expansion of about 0.000022 while the iron alloy has a co-efficient of thermal expansion of 0.000020.

Other proposals have involved, inter alia, the fitting of a light alloy piston with a piston ring carrier in the form of a steel ring of undefined thermal properties upon the head of a piston in such manner as to secure a positive lock with the body portion thereof, while in another case which extends to the provision of a light metal alloy piston with a ring located wholly above the upper compression ring or extending above the upper compression ring and being itself provided with a groove or grooves for the accommodation of the compression ring, it has been suggested to use a material such as a nickel-iron alloy having a low co-efficient of expansion to heat, that is to say, having a much smaller thermal co-efficient of expansion than the iron of which the cylinder is formed, and further, has a lower co-efficient of expansion to heat than the material forming the piston body, there being left between the ring and the adjacent portion of the body of the piston sufficient play so that the ring shall not be affected by the thermal expansion of the piston.

In another instance it has been suggested to employ gray cast iron or austenitic iron of particular compositions and it has been noted that where gray cast iron is employed to form a carrier for the compression rings and is arranged

to extend above the topmost compression ring groove that it is necessary to provide against any slackness arising in operation by forming the carrier ring with castellations, a similar construction being also desirable where austenitic iron having a co-efficient of expansion similar to that of the material forming the body of the piston is used.

The invention is based upon the observation that an unbroken ring of cast iron or steel of an austenitic character extending above the top of the compression ring and incorporated in the structure of the piston, in consequence of the relatively low rate of heat conductivity of austenitic iron and steel, and of the fact that it becomes surrounded by a film or skin of oxide in the casting of the body of the piston, operates to baffle the direct heat flow from the head of the piston to the topmost and the next succeeding row of grooves in which compression rings are arranged.

A further observation on which the invention is based is that the heat baffling effect may be secured by the incorporation in the piston of an insert at a position above the groove of the topmost compression ring even when the insert does not form a carrier for the upper compression ring or compression rings.

A further observation on which the invention is based is that austenitic iron or steel possessing a thermal co-efficient of expansion very considerably less than that of the light alloy may be employed in the formation of light alloy pistons having an aluminium or magnesium base in forming an insert or ring adjacent to the head of the piston and that, for instance, the difference of the co-efficient of expansion between the light metal alloy and the austenitic iron or steel may amount to 20% of the former.

The invention consists, broadly, in light alloy pistons for internal combustion engines and particularly for compression ignition engines in the structure of which is furnished an unbroken ring of cast iron or steel of an austenitic character at a position to function as a heat baffle between the head of the piston and the uppermost compression ring and having a co-efficient of expansion to heat which is more than 10% less than that of the light metal alloy and may be in the neighbourhood of 20% less than that of the light alloy.

Generally, the cast iron or steel of an austenitic character employed in accordance with the invention, has a thermal co-efficient of expansion of 0.000016 to 0.000019 per ° C. and generally

not greater than 0.000018, while the light metal alloy may have a co-efficient of expansion to heat at 20° C. of 0.000022 per ° C.

Tests have established that when the cooling of the piston with an insert of austenitic iron or steel takes place in the mould if the two materials have a similar co-efficient of expansion the grip on the width of the insert is very small, whereas a very definite contraction grip is obtained by the employment of austenitic iron or steel, in accordance with the invention, having a co-efficient of expansion to heat differing widely from that of the light metal alloy although the grip is within the elastic limit of the latter.

Thus, a very definite advantage is secured in that the insert is kept securely in position with the result that the risk of the insert becoming slack owing to inertia and general wear is minimised.

As an example of the composition of an austenitic cast iron which may be used in accordance with the invention, the following particulars are given:

|                                          |                |            |
|------------------------------------------|----------------|------------|
| Total carbon                             | percent        | 3.5        |
| Silicon                                  | do             | 2.0        |
| Phosphorus                               | do             | 0.2        |
| Manganese                                | do             | 0.9        |
| Nickel                                   | do             | 12 to 16.0 |
| Chromium                                 | do             | 2.25       |
| Copper                                   | do             | 6.0        |
| Co-efficient of expansion per ° C.       |                | .000018    |
| Ultimate tensile stress tons per sq. in. |                | 9/12       |
| Specific gravity                         |                | 7.686      |
| Heat conductivity                        | C. G. S. units | 0.10       |

Where, in accordance with the invention, the insert is in the form of an annulus which is provided with grooves for the accommodation of compression ring or rings, the annulus is preferably furnished on its inner face and adjacent to its upper extremity with a flange provided with one or more recesses leaving between the recesses radially extending projections.

For instance, such a ring may be of 185.25 mm. external diameter with a maximum internal diameter of 156.5 mm. and a diameter within the extremities of the flange of 148.5 mm. and in the flange are produced by means of a rotary cutter of circular form and 2" in diameter, recesses spaced apart from one another at an angle of 45°, the maximum depth of each of such recesses being equivalent to the width of the flange.

As above indicated, in accordance with the invention, the insert may be in the form of a ring or annulus which is not provided with recesses for the accommodation of compression rings.

In this case the ring or annulus is located in the piston above the level at which the compression rings are provided and it may extend into the piston head through a relatively considerable depth, that is to say, for a distance greater than that which an insert of the more usual form extends, and in this case the insert may also be relatively thin.

Conveniently, it is of dished or somewhat conical form with the portion directed to the apex extending away from the piston head.

With such a construction, while preferably austenitic cast iron or steel having a relatively low co-efficient of expansion is employed, the invention extends to the use of austenitic cast iron or steel such as has previously been proposed to be used in forming light metal alloy pistons with iron or steel inserts, or the composition of the light metal alloy may be varied so that its co-

efficient of expansion to heat corresponds more or less closely with that of the austenitic cast iron or steel employed.

The invention will be described further in detail and by way of example with reference to the accompanying drawings in which—

Figure 1 is a view in sectional elevation of one construction of piston in accordance with the invention,

Figure 2 is a view in sectional elevation of the insert therein,

Figure 3 being a view in sectional elevation on the line III—III of Figure 2,

Figure 4 being a plan view of the insert, while

Figure 5 is a view in sectional elevation of an alternative construction of piston in accordance with the invention.

Referring to Figures 1 and 5 of the drawings, in the body of the piston 1 which is formed in a light metal alloy and, for instance, an alloy having a content of 4 per cent. of copper, 2 per cent. of nickel, 1½ per cent. of magnesium, the balance being aluminium, the co-efficient of expansion to heat of which at 20° C. will be 0.000022 per ° C., adjacent to the head there is engaged a ring or annulus 2 formed of an austenitic cast iron of the composition and having a co-efficient of expansion of the character above indicated.

In the case of the construction shown in Figures 1, 2, 3 and 4, the annulus is provided with grooves 3 for the accommodation of compression rings on its outer face, and on its inner face it is furnished, adjacent to its upper extremity, with a flange 4, provided with a plurality of recesses 5 which leave between the recesses more or less radially extending projections, the recesses in the flange being produced by means of a rotary cutter of circular form.

In the case of a ring having an external diameter of 185.25 mm. the other dimensions thereof and the dimensions of the rotary cutter used in producing the recesses in the flange and its mode of use may be as indicated on the more general description given above.

In the case of the construction illustrated in Figure 5, the ring or annulus 2 is located above the level at which the topmost groove 6 for the accommodation of a compression ring is located and it extends into the body of the piston head through a relatively considerable distance, that is to say, for a distance greater than that which an insert of the more usual form would extend, the insert in the case of the construction illustrated being relatively thin and of dished or somewhat conical formation with the portion directed to the apex extending away from the piston head.

I claim:

1. A piston for an internal combustion engine comprising a cylindrical body portion formed of a light metal alloy and a ring of an iron alloy of an austenitic character engaged in the body portion at a position to function as a heat baffle between the head of the piston and the uppermost compression ring said iron alloy having a coefficient of expansion to heat which is between the limits of 10 per cent and 20 per cent less than that of the light metal alloy.

2. A piston for an internal combustion engine comprising a cylindrical body portion formed of a light metal alloy having a coefficient of expansion to heat in the neighbourhood of 0.000022 per degree centigrade at a temperature of 20° C. and a ring of an iron alloy of an austen-

itic character engaged in the body portion at a position to function as a heat baffle between the head of the piston and the position which the uppermost compression ring will occupy, said iron alloy having a coefficient of expansion to heat in the neighbourhood of and between 0.00016 and 0.000019 per degree centigrade.

3. A piston for an internal combustion engine, comprising a cylindrical body portion formed of a light metal alloy, a ring of an iron alloy of austenitic character embedded in said portion adjacent to the head thereof, said iron alloy having a coefficient of expansion to heat which is between the limits of 10 per cent and 20 per cent less than the coefficient of expansion to heat of the light metal alloy.

4. A piston ring for an internal combustion engine, comprising a cylindrical body portion formed of a light metal alloy, and an externally

grooved ring formed of an iron alloy of an austenitic character engaged in the said body portion adjacent to the head thereof, said iron alloy having a co-efficient of expansion to heat which is between the limits of 10 per cent and 20 per cent less than the coefficient of expansion to heat of the light metal alloy.

5. A piston for an internal combustion engine, comprising a cylindrical body portion formed of a light metal alloy, a ring of an iron alloy of austenitic character embedded in said portion adjacent to the head thereof and extending above the level at which the uppermost compression ring will be located, said iron alloy having a coefficient of expansion to heat which is between the limits of 10 per cent and 20 per cent less than the coefficient of expansion to heat of the light metal alloy.

ERIC BRADLEY GRAHAM.